

## UNITED STATES PATENT OFFICE

1,920,909

IRON OR STEEL AND PROCESS OF MAKING  
OR TREATING SAMEJoseph R. C. Marsh, Chicago, Ill., assignor to  
Francis N. Bard, Chicago, Ill.No Drawing. Application January 10, 1920  
Serial No. 350,549

2 Claims. (Cl. 75—45)

My invention relates to the manufacture of alloy steel, or to the treatment thereof during the manufacturing process or later operations thereon.

5 An object of my invention is to provide a treatment for iron or steel in the ladle, or crucible or other suitable retainer, which will impart thereto certain qualities which have not heretofore been obtained. Thus it is my object to increase the 10 toughness and tenacity of the iron or steel, to add to its tensile, torsional and transverse strength and at the same time to increase its strength in alternating stress and resistance to abrasion while keeping the compressive strength 15 high as well as the elastic limits high in all its strengths, and in short to make of the iron or steel a better product.

Other objects and advantages will appear herein.

20 In carrying my invention into effect I make use of copper and chromium with which the iron or steel is treated while in a molten state, with results as hereinafter described. The carbon, silicon, manganese, sulphur, phosphorus and other elements may be varied to meet certain requirements as in the case of other steels. The metallic copper raises the elastic limit and ultimate load in both steel and iron, gives resiliency 25 and to some extent hardness, and the chromium also adds to the ultimate load and gives the quality of resistance to shock or impact. The chromium and the copper both refine the grain. This alloy steel can be readily rolled, forged or otherwise mechanically formed.

30 My invention not only consists in making use of copper and chromium in the treatment of steel, but further consists in certain steps in this treatment found by me in practice to be necessary in view of certain novel conditions resulting 35 from the use of the above metals.

The copper can be added to the cold or molten charge or to the molten metal after the furnace begins to operate, sufficient time being allowed in the latter case to allow the copper to melt and properly mix with the molten metal. The chromium should be added preferably in the form of ferro-chromium after the manganese, or about fifteen minutes before pouring. The proportion 45 of ferro-chromium will depend upon its chromium content, so as to provide the chromium proportion of the formula in any instance.

50 As this alloy is difficult to weld, it becomes very important to properly deoxidize it. This should be done in the ladle or retainer in which it is made if direct pouring is practiced after the

alloy is made. This deoxidization is obtained by the addition of titanium, vanadium or boron, usually in the form of a ferro alloy. The silicon, manganese, carbon, phosphorus and sulphur contents are acquired according to the customary 60 methods.

As an example of the percentages of the elements which give good results, I may cite the following:

|                  | Percent |    |
|------------------|---------|----|
| Chromium about   | .85     | 65 |
| Copper about     | .85     |    |
| Silicon about    | .15     |    |
| Manganese about  | .25     |    |
| Sulphur about    | .03     |    |
| Phosphorus about | .03     | 70 |
| Carbon about     | .35     |    |
| Iron about       | 97.49   |    |

This table gives the proportion of the weight of each ingredient as compared with the total 75 weight of the complete resultant product. It will be understood that it is the treatment by adding the chromium and copper and the peculiar steps attending this treatment which distinguish my invention from heretofore known 80 processes of making or treating steel; and that a substance made up of any or all of the ingredients of the above list excepting the copper and chromium, or a substance including any other ingredient with iron such as to give it the ordinary properties of any of the well-known varieties of commercial alloy steel is to be considered 85 as a ferro metal alloy steel. Thus my formula according to the above example may be briefly stated as

|                   | Percent |  |
|-------------------|---------|--|
| Chromium about    | .85     |  |
| Copper about      | .85     |  |
| Ferro metal about | 98.30   |  |

An alloy manufactured substantially according 95 to the information above set forth is not merely useful in a cast form but is readily rolled into any of the usual shapes given to iron or steel; whereas any marked variation from the proportions of the elements, especially the copper and chromium, as herein given, precludes the mechanical working of this alloy as by rolling or forging, due to hot shortness, especially if the proportion of the copper is raised. This has been determined by me in actual practice.

To obtain an appreciable effect in accordance 100 with my invention, the copper and chromium should not be used in proportions much less than about .30% each. On the other hand, if much more than about 1.00% copper is used, the steel 110

is made so "hot short" that it cannot be successfully rolled; and if more than 3.00% of chromium be used the alloy steel will cost more than the increased results obtained from such excess 5 of chromium would justify.

The product is highly satisfactory in use where much more expensive steels have heretofore been found indispensable, as for instance, as tool steel, rails, car axles, tension members of railway cars 10 and bridges.

The superiority of my unheat treated alloy steel over open hearth steel has been demonstrated at the Bethlehem Steel Company at Bethlehem, Pennsylvania, as shown by its report of 15 September 17, 1919 in which eighty thousand pounds yield point in tension was obtained as against thirty-five thousand pounds customary yield point found in plain open hearth 40% carbon steel. Seven-eighths inch cold chisels made 20 of this steel have been driven through an inch of cold iron by being hammered with an eighteen pound sledge. The cutting edges and the striking ends of the chisels were not damaged.

It will be understood that while I have mentioned some uses for which my improved product 25 is most satisfactory and have specified certain ingredients and proportions of ingredients, in-

cluding those of the copper and chromium, in order to make a full and clear disclosure of my invention, nevertheless there is the possibility of some departure from the precise ingredients and proportions as well as many fields of usefulness not specifically mentioned herein, without departing from the scope or spirit of my invention, which, having thus fully set forth, I define in the following claims.

I claim:

1. The process of treating a ferro metal which consists in combining in a melted state such metal and copper, and afterward combining molten chromium with the combination of said metal and copper while said combination and the chromium are both in a melted state. 80

2. The method of treating a ferro metal which consists in combining in a melted state such metal and copper, then combining with the molten combination of said metal and copper a proper proportion of manganese while said combination and said manganese are in a melted state, and then combining with this combination chromium while this combination and said chromium are both in a melted state. 90 95 100

JOSEPH R. C. MARSH.

30

105

35

110

40

115

45

120

50

125

55

130

60

135

65

140

70

145

75

150